

## UNITED STATES PATENT OFFICE.

ERNEST CHARLES MORGAN, OF RICHMOND, ENGLAND.

## SENSITIVE PHOTOGRAPHIC-PRINTING PAPER.

SPECIFICATION forming part of Letters Patent No. 790,647, dated May 23, 1905.

Application filed December 22, 1904. Serial No. 238,014.

*To all whom it may concern:*

Be it known that I, ERNEST CHARLES MORGAN, manufacturer, a subject of the King of Great Britain, residing at Kew Foot road, 5 Richmond, in the county of Surrey, England, have invented certain new and useful Improvements in Sensitive Photographic-Printing Papers of the class known as "Self-Toning Printing-Out Papers" and the Like, of which 10 the following is a specification.

My invention relates to an improvement in sensitized photographic-printing papers, plates, and films, more especially of the class known as "self-toning" printing-out papers, 15 plates, and films," the invention consisting, essentially, in the employment as vehicle for the light-sensitive salts in the emulsion with which the support (paper, glass, celluloid, &c.,) is coated of agar-agar and arrowroot or other 20 suitable starch in substitution for gelatin or collodion. When paper is used as the support, it may be a pure raw paper or a paper with a baryta-coated surface, such as is in general use for photographic printing-out papers.

25 For a self-toning printing-out paper, the sensitive emulsion is made as follows: To twenty-four ounces of water add one and one-half ounces of arrowroot or other suitable starch and boil. In this mixture when cool 30 dissolve sugar, six drams; citric acid, five drams; ammonium chlorid, sixty-four grains; and Rochelle salt, four drams, and mix thoroughly. Add slowly nine drams thirty-six grains of nitrate of silver dissolved in eight 35 ounces of water. Next add slowly eleven grains of chlorid of gold dissolved in six ounces of water. Finally, take agar-agar two drams, boiled till dissolved in eighteen ounces of water, and add warm to the above mixture.

40 The paper, glass, celluloid, or other support is first coated with the above-described emulsion in a warm state and is then dried in a dark chamber. The sensitive paper or other material may thereafter be printed by expo- 45 sure to the action of light under a photographic

negative in the usual manner until a visible image of sufficient strength is obtained.

If a print of a purple-brown tone be required, the print is first washed for about ten minutes in running water and is then fixed 50 and toned in one operation by immersion for about fifteen minutes in a bath of hyposulfite-of-soda solution containing about twenty ounces of hyposulfite of soda to one hundred ounces of water. If a deeper purple tone be 55 required, then before washing the print or using the hyposulfite-of-soda bath the print is immersed for fifteen minutes in a bath containing twenty ounces of chlorid of sodium to one hundred ounces of water. 60

My reason for using agar-agar and arrowroot or other suitable starch as a medium in which to carry the light-sensitive salts instead of employing gelatin or collodion, which are the usual vehicles, is that in the case of self-toning 65 papers when gelatin is used as the vehicle the gold salt is not so easily reduced and will not give such satisfactory tones by immersion in hyposulfite-of-soda solutions only, while collodion as a vehicle is more costly. 70

I claim—

1. As a new article of manufacture a photographic printing-out paper, plate or film, comprising a support coated with a layer of a light-sensitive emulsion containing a mixture 75 of light-sensitive salts with agar-agar and starch.

2. As a new article of manufacture, a photographic-printing paper, plate or film, comprising a support coated with a light-sensitive 80 emulsion containing a gold salt, starch, and agar-agar.

3. As a new article of manufacture a photographic self-toning printing-out paper, plate or film, comprising a support coated with a 85 layer of a light-sensitive emulsion containing a mixture of light-sensitive salts and chlorid of gold with agar-agar and starch.

4. As a new article of manufacture, a photographic printing-out paper, plate or film, com- 90

prising a support coated with a mixture of aqueous solutions of starch, sugar, citric acid, ammonium chlorid, Rochelle salt, nitrate of silver and agar-agar.

5 5. As a new article of manufacture, a photographic self-toning printing-out paper, plate or film, consisting of a support coated with a mixture of aqueous solutions of starch, sugar,

citric acid, ammonium chlorid, Rochelle salt, nitrate of silver, chlorid of gold, and agar-<sup>10</sup> agar.

ERNEST CHARLES MORGAN.

Witnesses:

H. D. JAMESON,  
ALFRED NUTTING.